

Patented July 15, 1941

2,249,519

UNITED STATES PATENT OFFICE

YARN CONDITIONING PROCESS AND  
COMPOSITIONS THEREFOR

Joseph B. Dickey and James G. McNally, Rochester, N. Y., assignors to Eastman Kodak Company, Rochester, N. Y., a corporation of New Jersey

No Drawing. Application October 9, 1940,  
Serial No. 360,452

11 Claims.

(Cl. 28—1)

This invention relates to the conditioning of textile yarns and more particularly to the conditioning of filaments and yarns composed of organic derivatives of cellulose such as cellulose acetate, cellulose propionate, cellulose acetate propionate, and cellulose acetate butyrate to render them more amenable to textile operations such as knitting and the like.

As is well known in the manufacture of yarns, particularly those composed of or containing cellulose organic derivatives, it is necessary to treat the yarn in order to reduce the tendency toward breakage of the individual filaments or fibers when they are subjected to various mechanical strains and to lubricate the yarn in order to facilitate handling in such operations as spinning, twisting, winding and reeling. It is also necessary to treat yarn to adapt it for use as warp or filling or for the manufacture of various types of knitted fabrics. In knitting, it is particularly important that the yarn be soft and pliable in order that it may conform readily to the contour of the needles and thus produce a closely knit fabric free from such defects as "stitch distortion," "pin holes," "laddering," and the like.

Heretofore it has been proposed to employ softening agents such as polyhydric alcohols and similar agents as ingredients of yarn conditioning or lubricating formulas, generally in conjunction with mineral, animal or vegetable oils. It has been found, however, that most of the known softening agents and the various formulas containing them have certain drawbacks, one of the most serious of which is high vapor pressure, and in some cases too drastic a solvent action on the yarn. Many of such agents possess slight or insufficient solvent power for the lubricants with which they are used, and it is accordingly necessary to employ blending agents or emulsifying agents in order to obtain operable yarn treating formulas. In addition, many of the known softening and lubricating agents are insufficiently soluble in water to permit satisfactory removal by aqueous scour baths.

This invention has as its principal object to provide a new class of yarn conditioning agents particularly adapted for the conditioning of yarns composed of or containing organic derivatives of cellulose and capable of lubricating, softening and rendering such yarns more amenable to knitting and other textile operations. A further and specific object is to provide a class of conditioning agents which augment or assist the lubricating action of various lubricants when applied to such yarns. A still further object is to provide yarn softening and lubricating formulas which can be readily removed from the yarns by the usual scour baths. A still further object is to provide an improved method for the conditioning of yarns, particularly those composed

of or containing organic derivatives of cellulose such as cellulose acetate, whereby the yarn is rendered soft and pliable and capable of employment in a variety of textile operations where complicated designs or stitches are employed. Another object is to provide an improved type of yarn which is especially amenable to textile operations including circular knitting, weaving, spinning and the like. Other objects will appear hereinafter.

These objects are accomplished by the following invention which, in its broader aspects, comprises the discovery that ketals and acetals of tartaric acid having the general formula:



wherein R is a substituent selected from the group consisting of alkyl, cycloalkyl, aryl and heterocyclic groups, wherein R<sup>1</sup> and R<sup>2</sup> are substituents selected from the group consisting of hydrogen, alkyl, cycloalkyl, aryl and heterocyclic groups and wherein R<sup>3</sup> is a substituent selected from the group consisting of hydrogen, alkyl, cycloalkyl, aryl and heterocyclic groups may be used as yarn conditioning agents and particularly as softening agents, with or without the addition of animal, mineral, or vegetable oils, in the treatment of yarns composed of or containing organic derivatives of cellulose. We have found that these compounds when employed as described in the detailed examples set forth below have a slight solvent and/or softening action on cellulose organic derivative yarns which renders such yarns soft and pliable without at the same time having too drastic an action thereon. The alkyl group may be selected from methyl, ethyl, butyl, cyclo alkyl, benzyl, cetyl, ethoxyethyl, allyl and tetrahydrofurfuryl and the like. The aryl group may be phenyl, zenyl, naphthyl and furyl, etc. The heterocyclic group, for example, may be tetrahydrofurfuryl, morpholine, etc.

Typical compounds falling within the above classification may be prepared as described by Suzuki, Bull. Chem. Soc. Japan, 12, 487 (1937). This process of preparation may be extended to the preparation of derivatives of the above compounds.

In accordance with the invention these compounds may be applied directly to the yarn during or after spinning, or may be added to the spinning solution itself. We have found that these compounds have exceptional solvent powers which enable them to dissolve mineral oils and blown and unblown, drying and semi-drying, vegetable and animal oils and accordingly they may be, and preferably are, employed as ingredients of yarn conditioning or lubricating formulas in

conjunction with agents which function wholly or partially as lubricants.

In the following examples and description we have set forth several of the preferred embodiments of our invention, but they are included merely for purposes of illustration and not as a limitation thereof.

Our invention will be more readily understood by reference to the following examples in which typical applications of the invention are set forth.

*Example 1*



(Diethyl tartrate cyclohexyl ketal)

is applied to textile materials (silk, wool, cotton, cellulose acetate, viscose, etc.) by means of a bath, wick, roller, spray, etc. to facilitate their knitting, weaving, spinning and the like. If the yarn is intended primarily for knitting, the amount of conditioning liquid applied may vary from 2 to 25 per cent by weight of the yarn. If the yarn is intended primarily for weaving, the amount of conditioning liquid applied may vary between 1 and 5 per cent by weight of the yarn.

*Example 2*



(Diethyl tartrate naphthénal)

is applied to textile materials (silk, wool, viscose, cellulose acetate, etc.) from a benzene solution as in Example 1. The benzene is then removed by passing the materials through a suitable drying cabinet. If the yarn is intended primarily for knitting, the amount of conditioning liquid applied may vary from 2-25 percent by weight of the yarn. If the yarn is intended for weaving, the amount of conditioning liquid applied may vary between 1 and 5 percent by weight of the yarn.

*Example 3*

A conditioning liquid is made up as follows:

Olive oil..... Parts 99-1



(Oleyl methyl tartrate tetrahydrofural)

This is applied to textile materials such as silk, wool, cellulose acetate, etc., as described in Example 1. If the yarn is intended primarily for knitting, the amount of conditioning liquid applied may vary between 2 and 25 per cent by weight of the yarn, and if for weaving, the amount of liquid applied may vary between 1 and 5 per cent by weight of the yarn. Cellulose acetate filaments or fibers treated as described above are quite soft and pliable and give im-

proved results in various textile operations such as weaving, knitting, etc.

Compositions particularly useful for the conditioning of various types of yarns in accordance with our invention particularly those composed of or containing cellulose acetate, cellulose acetate propionate, cellulose acetate butyrate, and similar organic acid esters, are as follows:

*Example 4*



Parts 75-99

(Tetrahydrofurfuryl cetyl tartrate methyl butyl ketal)

Beta-methoxyethyl succinate..... 25-1

20

*Example 5*



75-99

(Di-beta-methoxy ethyl tartrate dinaphthénal)

Tetrahydrofurfuryl formal..... 25-1

30

*Example 6*



1-30

(Di-butyl tartrate butanal)

Blown olive oil..... 99-70

40

*Example 7*



1-40

(Cyclohexyl benzyl tartrate acetoneal)

Neat's-foot oil..... 99-60

50

*Example 8*



1-50

(Di-beta-ethoxy ethyl tartrate formal)

Blown neat's-foot oil..... 99-50

55

60

*Example 9*



1-89

(Dinaphthénal tartrate beta-methoxy-beta-ethoxy ethyl acetal)

75 Sperm oil..... 99-1

## Example 10

Glyceryl acetone acetate.....

Butyl naphthenate.....



(Beta-hydroxy ethyl ethyl tartrate acetal)

## Example 11

(Di-beta-methoxy ethyl tartrate methyl naphthyl ketal)  
Mineral oil.....(Di-beta-methoxy ethyl tartrate methyl naphthyl ketal)  
Blown neat's-foot oil.....Oleyl alcohol.....  
Tetrahydrofurfuryl tetrahydrofuroate.....

## Example 12

Mineral oil.....

Oleic acid.....



(Dinaphthyl tartrate beta-methoxy-beta-ethoxy ethyl acetal)

## Example 13

Mineral oil.....

Olive oil (blown or unblown).....

Oleic acid.....



(Oleyl potassium tartrate propanol)

Butyl stearate.....

## Example 14

Blown sperm oil.....

Mineral oil.....

Oleic acid.....



(Dinaphthyl tartrate-beta-methoxy-beta-ethoxy ethyl acetal)

Sodium sulfate.....

Oleic acid.....



## Example 15

## Example 16

Parts

10

20

5

10

10

10

10

10

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

15

yarn is intended for weaving, the amount may vary between about 1 and 5%.

Although in the above examples we have referred primarily to yarn treating compositions containing only the conditioning agent and an oil, other ingredients such as solvents, non-solvents, emulsifying agents, blending agents and the like, may be added within the scope of our invention. Likewise, various dyes or other coloring matter may be included in case it is desired to permanently or fugitively tint or dye the material undergoing treatment.

Although we have found it convenient to illustrate our invention by reference to compositions containing specific percentages of the various ingredients, these percentages may vary widely depending upon the particular purpose for which the composition is intended. For example, if it is desired to control the specific action of the conditioning agent, the amount of the agent may be adjusted as, for example, by reducing the amount of the agent and correspondingly increasing the amount of oil or other ingredient.

While we have described our invention with particular reference to the treatment of yarns composed of organic derivatives of cellulose such as cellulose acetate, the conditioning agents and formulas described herein are applicable to the conditioning of many other types of cellulose derivative yarns such as those composed of or containing cellulose propionate, cellulose butyrate, cellulose acetate propionate, cellulose acetate butyrate, ethyl cellulose, methyl cellulose, benzyl cellulose and others, as well as to the conditioning of silk, wool, cotton, viscose and other natural or artificial materials.

The term "yarn" as used herein and in the claims is to be understood as including a single filament, a plurality of filaments associated into the form of a thread, either of high or low twist, single or multiple threads associated or twisted together, composite threads composed of a mixture of natural and artificial filaments or a composite thread formed by twisting together individual strands of natural or artificial materials, as well as cut staple fibers produced from natural and/or artificial filaments or threads and spun yarn produced from such staple fibers.

The yarn conditioning method and compositions of our invention possess many outstanding advantages. The fundamental and outstanding characteristic of the agents employed in accordance with the invention is their ability to soften yarns, especially those composed of or containing organic derivatives of cellulose such as cellulose acetate and render them soft and pliable and amenable to various textile operations, especially operations such as those involved in weaving and knitting where complicated designs or stitches are employed, without too drastic an action on the yarn material. Another outstanding characteristic of these compounds is their exceptional solvent power for a wide variety of mineral, animal, and vegetable oils and their ability to act as lubricating assistants in conjunction with these oils when applied to such yarns. In addition, due to their solubility in water, they may be readily removed from yarns and fabrics by means of the usual aqueous scour baths. By employing the yarn conditioning agents and method of our invention as herein described, one is enabled to obtain highly satisfactory results in the manufacture of yarns and woven fabrics and especially

the production from these yarns of closely knit fabrics free from defects such as pin holes, stitch distortion, ladder and the like.

Of the above compositions we have found that di-beta-ethoxy ethyl tartrate formal, cyclohexyl benzyl tartrate acetoneal and dibutyl tartrate butanal are outstanding in their ability to lubricate and soften yarns composed of or containing organic derivatives of cellulose and render them amenable to a wide variety of textile operations, particularly knitting.

What we claim is:

1. The process of conditioning yarn to render it more amenable to textile operations including knitting, weaving, spinning and the like which comprises applying thereto a lubricating and softening composition containing as its essential lubricating and softening component a compound selected from the group consisting of the ketals and acetals of tartaric acid having the general formula:



wherein R is a substituent selected from the group consisting of alkyl, cycloalkyl, aryl and heterocyclic groups, wherein R<sup>1</sup> and R<sup>2</sup> are substituents selected from the group consisting of hydrogen, alkyl, cycloalkyl, aryl and heterocyclic groups and wherein R<sup>3</sup> is a substituent selected from the group consisting of hydrogen, alkyl, cycloalkyl, aryl and heterocyclic groups.

2. The process of conditioning yarn composed of or containing organic derivatives of cellulose to render it more amenable to textile operations including knitting, weaving, spinning and the like which comprises applying thereto a lubricating and softening composition containing as its essential lubricating and softening component a compound selected from the group consisting of the ketals and acetals of tartaric acid having the general formula:



wherein R is a substituent selected from the group consisting of alkyl, cycloalkyl, aryl and heterocyclic groups, wherein R<sup>1</sup> and R<sup>2</sup> are substituents selected from the group consisting of hydrogen, alkyl, cycloalkyl, aryl and heterocyclic groups and wherein R<sup>3</sup> is a substituent selected from the group consisting of hydrogen, alkyl, cycloalkyl, aryl and heterocyclic groups.

3. The process of conditioning yarn composed of or containing cellulose acetate to render it more amenable to textile operations including knitting, weaving, spinning and the like, which comprises applying thereto a lubricating and softening composition containing as its essential lubricating and softening component a compound selected from the group consisting of the ketals and acetals of tartaric acid having the general formula:



wherein R is a substituent selected from the group consisting of alkyl, cycloalkyl, aryl and heterocyclic groups, wherein R<sup>1</sup> and R<sup>2</sup> are substituents selected from the group consisting of hydrogen, alkyl, cycloalkyl, aryl and heterocyclic groups and wherein R<sup>3</sup> is a substituent

selected from the group consisting of hydrogen, alkyl, cycloalkyl, aryl and heterocyclic groups.

4. The process of conditioning yarn composed of or containing cellulose acetate to render it more amenable to textile operations including knitting, weaving, spinning, and the like, which comprises applying thereto a lubricating and softening composition containing as its essential lubricating and softening component di-beta-ethoxy ethyl tartrate formal.

5. The process of conditioning yarn composed of or containing cellulose acetate to render it more amenable to textile operations including knitting, weaving, spinning and the like, which comprises applying thereto a lubricating and softening composition containing as its essential lubricating and softening component cyclohexyl benzyl tartrate acetoneal.

6. The process of conditioning yarn composed of or containing cellulose acetate to render it more amenable to textile operations including knitting, weaving, spinning and the like, which comprises applying thereto a lubricating and softening composition containing as its essential lubricating and softening component dibutyl tartrate butanal.

7. Textile yarns amenable to textile operations including knitting, weaving, spinning and the like impregnated with a lubricant containing as its essential lubricating and softening component a compound selected from the group consisting of the ketals and acetals of tartaric acid having the general formula:



wherein R is a substituent selected from the group consisting of alkyl, cycloalkyl, aryl and heterocyclic groups, wherein R<sup>1</sup> and R<sup>2</sup> are substituents selected from the group consisting of

hydrogen, alkyl, cycloalkyl, aryl and heterocyclic groups and wherein R<sup>3</sup> is a substituent selected from the group consisting of hydrogen, alkyl, cycloalkyl, aryl and heterocyclic groups.

5. 8. Textile yarns composed of or containing organic derivatives of cellulose amenable to textile operations including knitting, weaving, spinning and the like, impregnated with a compound selected from the group consisting of the ketals and acetals of tartaric acid having the general formula:



15 wherein R is a substituent selected from the group consisting of alkyl, cycloalkyl, aryl and heterocyclic groups, wherein R<sup>1</sup> and R<sup>2</sup> are substituents selected from the group consisting of hydrogen, alkyl, cycloalkyl, aryl and heterocyclic groups and wherein R<sup>3</sup> is a substituent selected from the group consisting of hydrogen, alkyl, cycloalkyl, aryl and heterocyclic groups.

20 9. Textile yarns composed of or containing cellulose acetate amenable to textile operations including knitting, weaving, spinning and the like, impregnated with a lubricant comprising di-beta-ethoxy ethyl tartrate formal.

10. Textile yarns composed of or containing cellulose acetate amenable to textile operations including knitting, weaving, spinning and the like, impregnated with a lubricant comprising cyclohexylbenzyl tartrate acetoneal.

11. Textile yarns composed of or containing cellulose acetate amenable to textile operations including knitting, weaving, spinning and the like, impregnated with a lubricant comprising dibutyl tartrate butanal.

40

JOSEPH B. DICKEY,  
JAMES G. McNALLY.